

# United States Patent [19]

Lulay et al.

[11] 4,324,095

[45] Apr. 13, 1982

[54] **PROCESS FOR PREPARING SLUB YARNS**

[75] Inventors: Arthur Lulay, Wilmington, Del.; Charles E. Lynch, Camden, S.C.

[73] Assignee: E. I. Du Pont de Nemours and Company, Wilmington, Del.

[21] Appl. No.: 868,488

[22] Filed: Jan. 11, 1978

[51] Int. Cl.<sup>3</sup> ..... D02G 3/00; D02G 3/34

[52] U.S. Cl. ..... 57/327; 57/209; 57/254; 57/256; 57/317; 428/359; 428/373; 428/399

[58] Field of Search ..... 428/373, 359, 374, 370, 428/364, 399, 400; 57/139, 140 J, 140 BY, 156, 157 R, 209, 206, 327, 317, 254, 256; 19/145.5, 145.7, 98

[56] **References Cited**

**U.S. PATENT DOCUMENTS**

3,007,227 11/1961 Moler ..... 428/359 X  
3,038,237 6/1962 Taylor, Jr. ..... 428/370

3,038,238 6/1962 Wu ..... 428/394 X  
3,038,239 6/1962 Moulds ..... 264/171 X  
3,038,240 6/1962 Kovarik ..... 428/371 X  
3,039,524 6/1962 Belck et al. ..... 428/374  
3,092,892 6/1963 Ryan, Jr. et al. ..... 428/394 X  
3,103,098 9/1963 Dyer ..... 428/399 X  
3,161,011 12/1964 Humphreys ..... 28/281 X  
3,350,872 11/1967 Gorrafa ..... 57/140 BY X  
3,429,017 2/1969 Hofeld ..... 57/140 BY  
3,626,684 12/1971 Hovis ..... 57/140 BY  
3,663,676 5/1972 Lulay ..... 264/168  
3,841,078 10/1974 Hartsog ..... 428/364 X

Primary Examiner—Lorraine T. Kendall

[57]

## ABSTRACT

Slub yarns are prepared by adding 10–50% by weight 0.25 to 1 in. long bicomponent acrylic fibers having a density of about 1.0 to 1.17 g/cm<sup>3</sup> and an equilibrium crimp reversibility of at least about 20% with staple fibers during or before carding and processing to a slab containing spun yarn in a conventional manner.

11 Claims, 2 Drawing Figures





FIG. 1

FIG. 2

## PROCESS FOR PREPARING SLUB YARNS

This invention relates to an improved process for preparing slub yarns by adding nubs of short bicomponent acrylic fibers to staple fibers during or before carding and processing the resulting fiber blend by conventional methods to produce a slub yarn. When woven or knit into fabrics, the slub yarns produce desirable visual effects.

It is known to produce effect yarns by adjustment of a card to produce a certain amount of rolling of the staple fibers fed which rolls some of the shorter fibers into balls which are not drafted out during carding and subsequent processing. The resulting yarn has a degree 15 of non-uniformity with respect to diameter which can produce a pleasing visual effect when suitably knit or woven into a fabric. It is also known that if yarns containing larger nonuniformities are desired, such yarns are conveniently prepared by adding nubs (knops) of 20 short rayon fibers to staple fibers before or during carding and to process the resulting fiber blends into spun yarns containing slubs. However, these rayon nubs are relatively expensive to produce and have different dyeing characteristics than many synthetic fibers.

Because of their high resistance to degradation on exposure to ultra violet light, acrylic fibers are eminently suited for use in curtains and draperies. Slub yarns of acrylic fibers which are suitable for weaving into fabrics resembling antique satins are highly desired. 30 Such acrylic fibers are also favored for use in knit goods such as sweaters.

## SUMMARY OF THE INVENTION

This invention provides an improved process for 35 preparing slub yarns suitable for the preparation of knit and woven fabrics having desirable visual effects.

This invention provides an improved process for producing a slub yarn wherein 10-50% by weight bicomponent acrylic fibers having a hydrophilic component and a less hydrophilic component and having a density of about 1.0 to 1.17 g./cm<sup>3</sup> and an equilibrium crimp reversibility of at least about 20% and cut to a length of 0.25 to 1 inch are blended with staple fibers in 40 an amount of 50-90% by weight during or before carding and processed by conventional procedures into a slub containing spun yarn. One component of the bicomponent acrylic fibers is hydrophilic and is preferably comprised of (1) 85-98% by weight acrylonitrile units, (2) 2-10% by weight units of styrene sulfonic acid (o-, m- or p- isomer), 2-acrylamido-2-methylpropane sulfonic acid, allyl sulfonic acid, methallyl sulfonic acid, vinyl sulfonic acid, or their metal, ammonium or amine salts, a vinyl pyridine, vinyl pyrrolidone, acrylamide, methacrylamide, hydroxymethylacrylamide or mixtures thereof, (3) 0 to 13% by weight of units of a comonomer less hydrophilic than units of monomer (2). The other component of the bicomponent fibers is less hydrophilic and preferably contains 0-20% by weight of a polymer as described above and 80-100% by weight 45 polyacrylonitrile. Preferably the less hydrophilic comonomer (3) is methyl acrylate, methyl methacrylate, vinyl acetate, methacrylonitrile or mixtures thereof. The process is preferably carried out on the cotton or worsted spinning systems. The bicomponent fibers preferably have a length of 0.25 inches when used on the cotton system and a length of 0.75 inches when used on the worsted system. In a preferred embodiment of the

invention a card sliver containing bicomponent acrylic fibers according to the invention is blended with one or more card slivers which do not contain such bicomponent acrylic fibers. Improved effects can be obtained 5 when the bicomponent acrylic fibers are coated with a high friction finish.

## DRAWINGS

FIG. 1 is a front elevational view of a holder used to 10 measure equilibrium crimp reversibility (ECR).

FIG. 2 is a side elevational view of a holder used to 15 measure ECR.

## DETAILED DESCRIPTION OF THE INVENTION

The bicomponent acrylic fibers used in the present invention may be cut from the tow described in copending application No. 681,592 filed Apr. 29, 1976. This application describes tows of highly entangled, continuous, eccentric bicomponent acrylic filaments in which the filaments have a density of 1.0-1.17 g./cm<sup>3</sup>, an equilibrium crimp reversibility (ECR) of at least about 20% and a filament entanglement value greater than about 12 and less than about 60. The tows are prepared by drying 25 a previously undried tow of continuous acrylic filaments having an eccentric bicomponent structure in which a large difference exists between the hot water swellability of the components of the filaments as indicated by their equilibrium crimp reversibility (ECR). 30 The drying is carried out at a temperature below the hot-wet glass transition temperature (T<sub>g</sub>) of the fiber polymers until the moisture content of the tow is no more than 3% by weight. The tows may be cut to the desired length by any convenient method such as by using a Lummus cutter.

Alternatively, a wet, never-dried, tow of continuous, eccentric, bicomponent acrylic filaments having an equilibrium crimp reversibility (ECR) of at least about 20% may be cut to the desired length and then dried at 35 a temperature below the hot-wet glass transition temperature (T<sub>g</sub>) of the fiber polymers.

The optimum length of the bicomponent fibers suitable for use in the present invention within the range of 0.25 to 1 inch depends on the system used to prepare the slub yarn. When the cotton system is used, the preferred length of the bicomponent fibers is 0.25 inches. On the other hand, when the worsted system is used, the optimum length of the bicomponent fibers is 0.75 inches.

The bicomponent acrylic fibers have a large difference in the hot water swellability of the two components. Such bicomponent acrylic fibers are described in U.S. Pat. No. 3,092,892 issued June 11, 1963. The difference in hot water swellability of the components making up the bicomponent fibers is measured as equilibrium crimp reversibility (ECR). By "hot" water is meant that the water has a temperature in the region of from about 70° C. up to about the boiling point of water. A higher (ECR) reflects a higher differential between the dry and wet length of the fiber components. While the fibers can have an ECR higher than about 60%, such fibers are not easily prepared on a commercial basis. However, a minimum ECR of about 20% is necessary to obtain the minimum differential in the swellability of the fiber components which will provide adequate crimp development to sufficiently entangle the fibers. Fibers having an ECR of about 20-60% exhibit pronounced differential crimp changes ("squirm") on

drying. This arises because the fibers comprise two components in a substantially eccentric relationship in the sense that the cross sections of the components have center points that do not coincide. Such fibers generally develop a pronounced helical crimp on relaxed exposure to conditions that permit relief of stresses imparted during manufacture. Within a most preferred range of ECR of about 30-50%, optimum helical crimp is developed on drying, thus providing optimum fiber entanglement.

The eccentric bicomponent fibers useful in the present invention develop a high helical crimp amplitude, and therefore have a high crimp index. A crimp index of about 10-40, preferably about 20-30, characterizes the fibers useful in the present invention. The higher crimp amplitude is believed to enhance entanglement. At a crimp index of about 20-30, optimum crimp amplitude to provide concomitantly optimum entanglement is obtained. The bicomponent fibers useful in the present invention have a crimp frequency of about 2-15 crimps/cm of extended fiber length. When the more hot water swellable component is situated on the inside of the crimp helices, the fiber loses some of its crimp under hot-wet conditions and regains it on drying. The reverse occurs when the more hot water swellable component is on the outside of the crimp helices. Hence, when the more hot water swellable component is on the inside in the dry state, adequate crimp development occurs on drying and fiber has a positive ECR.

Hot water swellability is enhanced by incorporating in the bicomponent fiber polymers units of ionizable monomers which confer dye receptivity to the polymers as illustrated in Taylor U.S. Pat. Nos. 3,038,237 and 3,039,524. Non-ionic monomers that confer hot water swellability to the fiber components include acrylamide, methacrylamide and the betaines as illustrated in U.S. Pat. Nos. 3,470,060 and 3,473,998. Blends of an acrylic polymer and a highly hot water swellable polymer can also be used as discussed in U.S. Pat. No. 3,038,239. The composite fibers described in U.S. Pat. No. 3,092,892 are particularly suitable for use in the present invention.

Any two polymeric components disclosed in the patents referred to above which have a substantial difference in hot water swellability can be used to make the eccentric bicomponent acrylic fibers to be used in the present invention with the proviso that the components possess a difference in hot water swellability which provides the fibers with an ECR of at least about 20%, preferably about 20-60%. Two or more polymers may also be employed as one or each of the two components.

Preferred polymers or blends of polymers which can function as the fiber component having lower hot water swellability include those comprising (A) about 80-100% by weight of a polymer comprising about 85-100% by weight of units derived from acrylonitrile and 0 to about 15% by weight of units derived from a monomer copolymerizable with acrylonitrile and which is less hydrophylic than a monomer of (2) below including methyl acrylate, methyl methacrylate, vinyl acetate, methacrylonitrile and the like and mixtures thereof, and (B) about 20-0% by weight of a polymer comprising (1) about 85-98% by weight of units derived from acrylonitrile, (2) about 2-10% by weight of units derived from one or more of styrene sulfonic acid (o-, m- or p-isomer), 2-acrylamido-2-methylpropane sulfonic acid, allyl sulfonic acid, methallyl sulfonic acid,

v vinyl sulfonic acid, or their metal, ammonium or amine salts, a vinyl pyridine, such as 2-vinyl pyridine or 2-methyl-5-vinyl pyridine, vinyl pyrrolidone, acrylamide, methacrylamide, hydroxymethylacrylamide and the like and mixtures thereof and (3) 0 to about 13% by weight of units derived from any other copolymerizable monomer known in the art which is less hydrophilic than units of a monomer of (2), including methyl acrylate, methyl methacrylate, vinyl acetate, methacrylonitrile and the like and mixtures thereof.

The bicomponent acrylic fibers prepared as described in the patents mentioned herein reach most of their full helical crimp capability during drying at a temperature below the hot-wet glass transition temperature ( $T_g$ ) of the fiber polymers. Typically, more crimp (than is achieved with high-temperature dried fibers only after boil-off or steaming after-treatments) is developed in the bicomponent fibers useful in the present invention when they are dried at a temperature below the  $T_g$  of the fiber polymers, without the need for such after-treatment. However, even higher crimp can be achieved in the low density fibers useful in the present invention by such after-treatment, especially if carried out under little restraint, as when boiling off chips of cut tow. In addition, the density of the dried fibers is strictly dependent on the drying temperature. Generally, temperatures of about 30-80° C., preferably about 50-70° C., are used depending on the polymer structure, the degree of orientation and the kind of treatment to which the undried fibers have been subjected which might change the  $T_g$  of the polymer and the filaments. The preferred range provides optimum results in terms of time and cost. At temperatures above the  $T_g$  of the fiber polymers, e.g., about 80° C., the water escapes while the fiber is too limp to develop adequate crimp and entanglement, and the fiber structure can compact, resulting in a high density fiber. At a temperature much below about 30° C., the drying operation is commercially undesirable since it requires a very high flow of drying medium and a long hold-up time. Air or any other gas inert to the fibers may be used as the drying medium. On the other hand, a solvent that extracts water may be used or vacuum may be applied.

Additional treatments such as steaming, boil-off and so on may be employed to further optimize the properties of the bicomponent acrylic fibers useful in the present invention.

The short bicomponent acrylic fibers may be added to the other fibers during or before carding. For example, they can be added during opening or during a mixing step. When large slubs are desired, it is advantageous to prepare a sliver containing a higher concentration of the short bicomponent fiber that is ultimately desired and then to blend this sliver with one or more other slivers which do not contain the short bicomponent acrylic fibers suitable for use in the present invention.

The slub yarns are prepared under normal processing conditions on the cotton or worsted systems. Combing is omitted since this would tend to remove the slubs. The bicomponent acrylic fibers may be blended with any staple fibers suitable for processing in the desired system.

## TEST METHODS

## Equilibrium Crimp Reversability (ECR)

Tows of dried, crimped filaments to be tested are cut to chips of about 10 cm crimped length and the chips are given a relaxed, 30-minute boil-off loosely wrapped in a single thickness of chessecloth. They are dried for 30 minutes in an oven at 70° C.

Fibers are selected randomly from the boiled off and dried chips and mounted in holders designed to measure ECR as illustrated in the Figures in which like numerals refer to the same element. In the figures, holder base 10 is a sheet of black plastic about 3.8 cm wide, 0.6 cm thick and 20 cm long. Three blocks of aluminum 20, 21 and 22 about 1.3 cm square and 3.8 cm long are firmly attached to one face of the base. The first block 20 is attached across the bottom end of base 10. Another block 21, attached across the top end of base 10 is drilled through its center and parallel to the length of base 10 to just allow an 18 cm long, fully threaded rod 30, approximately 0.6 cm in diameter to pass through. The third block 22 is drilled similarly to block 21, except that it is threaded and positioned about 8 cm above bottom block 20. The diameter of rod 30 is reduced on a lathe at each end 31, 32 to about 0.3 cm for a length of about 0.8 cm. A knurled knob 33 is securely attached to end 31. A fourth aluminum block 23 of the same dimensions as the three mounted blocks is movable and is drilled from the center of one face to pass freely end 32 of threaded rod 30. From one face the hole is counter-drilled to give a counterbore 27 of about 0.6 cm diameter and about 0.7 cm depth, leaving a flat bottom. A disc of aluminum 40 about 0.16 cm thick and about 6.3 cm in diameter is drilled through its center to pass the threaded rod and is firmly attached to the top of aluminum block 21 to serve as a hanger for the holder.

The apparatus is assembled by passing the free end of threaded rod 30 through aluminum disc 40 and top block 21, screwing it through threaded block 22, and passing end 32 through the loose block 23 so that it terminates in counterbore 27 where it is secured with compression washer 28, leaving enough clearance to permit free turning of rod 30. By turning knob 33, movable block 23 is positioned approximately 5 cm from bottom block 20.

One end of each of five boiled-off and dried fibers is taped to movable block 23. The other ends are then taped to bottom block 20 after pulling out slack but not crimp, using care to leave about the same crimped length of fibers between the blocks. Holder base 10 is labeled to identify the sample, and movable block 23 is moved down to provide definite slack in the fibers.

When the required number of fibers have been loaded into holders, the required number of the holders are placed for at least 30 minutes in a glass-walled bath of water maintained at 70° C. Movable block 23 of each holder is moved upward to remove slack from the fibers, and the wet crimp therein counted using a cathetometer; each convexity on one side of the fiber is regarded as a crimp.

The holders are removed from the bath; fiber slack is re-established by moving block 23 downward; the holders are placed in a 70° C. oven for about thirty minutes and then stored at room temperature (about 21° C., 65% relative humidity) for 30 minutes. Dry crimps are counted as described above after removing slack.

$$ECR = \frac{(No. \text{ of crimps dry} - No. \text{ of crimps wet})}{No. \text{ of crimps dry}} \times 100\%$$

5 Determinations on about 100 fibers are required for good reliability.

10 Density is determined in carbon tetrachloride/heptane density gradient tubes prepared as known in the art. The range from 1.00 to 1.22 g/cc is covered by two tubes (standard 250 ml graduated cylinders). For the first, the following "stock" solutions are prepared from well-dried solvents:

|    | ml               |         | Approx. density |
|----|------------------|---------|-----------------|
|    | CCl <sub>4</sub> | heptane |                 |
| 27 | 56               | 0.980   |                 |
| 29 | 54               | 1.002   |                 |
| 31 | 52               | 1.023   |                 |
| 33 | 51               | 1.041   |                 |
| 34 | 49               | 1.056   |                 |
| 36 | 47               | 1.077   |                 |
| 38 | 45               | 1.099   |                 |
| 40 | 43               | 1.120   |                 |

15 The second is prepared from the following "stock" solutions:

|    | ml               |         | Approx. density |
|----|------------------|---------|-----------------|
|    | CCl <sub>4</sub> | heptane |                 |
| 38 | 45               | 1.099   |                 |
| 40 | 43               | 1.120   |                 |
| 42 | 42               | 1.137   |                 |
| 43 | 40               | 1.153   |                 |
| 45 | 38               | 1.174   |                 |
| 47 | 36               | 1.196   |                 |
| 49 | 34               | 1.217   |                 |
| 51 | 33               | 1.232   |                 |

20 To prepare the tubes, 30 ml of the densest stock solution is poured into a 250-ml graduate, followed by 30 ml of the next lighter solution, and the others in turn, until 30 ml of each of the solutions has been added. The second and all subsequent additions are made slowly through a pipette, holding the tip near the wall of the cylinder, to avoid mixing. The two cylinders are placed in a water bath controlled at 25° ± 0.1° C. and clamped securely in a vertical position. The tubes are stoppered except when making additions or removals.

25 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 87

54% bicomponent basic dyeable acrylic staple fibers and 36% by weight acid dyeable acrylic fiber. The samples are prepared by hand blending the component fibers in the hopper of a card without attempting to break up the nubs of short bicomponent acrylic fibers into smaller clumps. The components are:

A. 10 Parts—6 dpf (0.67 tex) 0.5 or 0.25 inch (0.635 or 1.27 cm) (length bicomponent filaments)

B. 54 Parts—Commercial 6 dpf (0.67 tex) varicut to 4.5–6 inches (11.4–15.2 cm.) length

Acrylic bicomponent staple fibers of the differential component swellability type taught in U.S. Pat. No. 3,092,892.

C. 36 Parts—Commercial 8.5 dpf (0.94 tex) varicut to 3–5.5 inches (7.6–14 cm.) length acrylic, acid-dyeable bright, low-crimp, surface modified (for softness) staple fibers of the type disclosed in U.S. Pat. No. 2,891,035 containing 88.8% by weight acrylonitrile, 5.8% by weight methyl acrylate and 5.9% by weight methyl vinylpyridine.

Carding of each on a 72 inch (183 cm.) single-cylinder Davis and Furber Card provided a somewhat clumpy 390 gr. (27,650 tex) sliver which was twice servo pin drafted with 10 ends fed, using 9 pins/inch (3.5 pins/cm.) and twice more pin drafted with 4 ends fed, using 15 pins/inch (6 pins/cm.) to yield a 110 gr. (7800 tex) sliver. A slubber was used to make a 20 gr. (1420 tex) roving with 0.4 twist/inch (0.16/cm.), which was spun on a spinning frame to make 3 items. Item a is made from sliver containing 0.5 inch bicomponent acrylic fibers and items b and c are made using sliver containing 0.25 inch bicomponent acrylic fibers.

| Worsted Count        | twist/inch (cm.) | Spindle Speed (rpm) | Scott Skein Strength lbs (kg) singles |
|----------------------|------------------|---------------------|---------------------------------------|
| a. 4/7.5 (4/472 tex) | 3.8 (1.5)        | 4000                | 252 (~114)                            |
| b. 2/12 (2/148 tex)  | 5.3 (2.1)        | 4500                | 182 (~83)                             |
| c. 2/20 (2/88 tex)   | 8.2 (3.2)        | 5000                | 106 (~48)                             |

The fly level and ends down were higher for these items than for uniform-tex yarns, but not prohibitively so.

When these yarns were cross-dyed with a mixture of basic and acid dyes, attractive novelty slab yarns were obtained in which the slubs differed in color from the background.

## EXAMPLE II

### Worsted System

Following the procedures of Example I, the following were hand weighed and double-blended on an opener.

15 parts of Component A of Example I, 0.5 inches (1.27 cm.) in length

52.5 parts of Component B of Example I

32.5 parts Component C of Example I

Carding at 150 lbs./hour (68 kg./hr.) on a Davis and Furber card yielded a 350 gr. (24,850 tex) sliver without excessive static, cylinder loading or fiber fall-out (about 3%).

Drafting in 3 stages first on a Warner and Swazey servo with eight ends fed, using 12 pins/inch (4.7/cm.) then, intermediate and finisher each with 4 ends fed, using 18 pins/inch (7.1/cm.) ran smoothly to give 100 grain (7100 tex) sliver with 6% CV. By comparison, a similar yarn containing 10% by weight rayon nubs in-

5 stead of component A had a CV, or coefficient of tex variation of 4.5% by weight.

The slubbing operation ran smoothly to give a roving of 13% CV (versus 9.5–10% for a comparable roving using rayon nubs). Spinning was at a 5,000 rpm spindle speed to give a 1/12 worsted count (74 tex) 7 turns per inch yarn of adequate (232 pounds [105 kg] Scott-skein) strength. Performance was judged adequate, although both fly and breaks were somewhat higher than normal. Yarn quality, after plying to 2/12 worsted count (148 tex) was judged acceptable for novelty end uses and gave attractive slab sweaters when cross-dyed as in Example I.

The slubs were significantly larger and longer than those obtained in ordinary cotton-system processing, as were the slubs obtained in the yarns of Example I.

The same blend levels and spinning process was used to evaluate small lots comprising 15% of the 6 dpf (0.67 tex) nubs of component A which differed in length. They were 0.25, 0.5, 0.75 and one inch in length or a blend of 66% 0.5 inch length and 34% one inch length fibers. Textile performance, as measured by efficiency and uniformity of pin drafting, the number of spinning ends down, overall performance in spinning and plying, improved with increasing lengths of the bicomponent fiber. The yarns were evaluated by winding each on a mirror board and rating them in terms of frequency and size of the slubs. The length and frequency of slubs in the yarns increased with increasing bicomponent fiber length in this comparison, but the best balance of spinning performance and acceptable slab appearance (frequency and large size) was realized with 0.75 inch bicomponent fibers. No special advantage was found in use of the blend of nubs of different lengths.

## EXAMPLE III

This example illustrates a means to increase the length and thickness of slubs in a yarn using the cotton system. The yarn preparations were based on a blend of 85 parts of a commercial acrylic 3-denier/filament (~0.33 tex), 2-inch (~5 cm.) bright, trilobal staple intended for cotton-system processing to yarns for knitwear and 15 parts of 0.25 inch (~0.6 cm.) 6 denier/filament (~0.67 tex) nubs of this invention blended before picking. They were prepared: I. without modification of the process or equipment; II. after spraying onto the nubs 3% (non-volatiles) of a finish containing the triethanolamine salt of a C<sub>6</sub>–C<sub>8</sub> alcohol partial ester of phosphoric acid, boric acid, diethylene glycol, triethanolamine and a commercial nonionic surfactant to raise the level of fiber-to-fiber friction, without further modification; III. no modification except that a card sliver containing 30% by weight of the 0.25 inch long bicomponent fibers was blended to 15% nubs in drafting. IV. This item is a commercial item with 15% rayon slubs useful in preparing antique satin fabrics, for comparison.

Each 8/1 cotton count (~74 tex) yarn was analyzed on a Uster Classimat. Results are summarized in the Table below, the frequency of slubs per 100,000 yds. (91,400 m) being tabulated in the Classimat manner. In these classifications, the slab length increases from A (~1.0 cm.) to D (~4.0 cm.) and slab diameter increases 1 (~100%–150% larger than base yarn) to 4 (~400% larger than the base yarn).

| Classi-<br>mat | Normal | I<br>High-Frict<br>Finish | II<br>High bicomponent<br>Fiber Card<br>Concentration | III              |    |
|----------------|--------|---------------------------|-------------------------------------------------------|------------------|----|
|                |        |                           |                                                       | IV<br>Comparison |    |
| A-1            | 12,164 | 10,708                    | 12,216                                                | 84,768           |    |
| A-2            | 884    | 742                       | 326                                                   | 17,112           |    |
| A-3            | 12.1   | 11                        | 5                                                     | 356              |    |
| A-4            | 0      | 6                         | 5                                                     | 4                |    |
| B-1            | 3,325  | 5,089                     | 21,856                                                | 23,725           |    |
| B-2            | 917    | 1,253                     | 4,776                                                 | 21,943           | 10 |
| B-3            | 73     | 60                        | 109                                                   | 2,220            |    |
| B-4            | 6      | 11                        | 6                                                     | 3                |    |
| C-1            | 760    | 1,836                     | 9,259                                                 | 6,132            |    |
| C-2            | 314    | 797                       | 6,334                                                 | 9,823            |    |
| C-3            | 48     | 61                        | 469                                                   | 2,356            |    |
| C-4            | 7      | 62                        | 46                                                    | 136              |    |
| D-1            | 72     | 407                       | 1,973                                                 | 594              | 15 |
| D-2            | 45     | 413                       | 3,474                                                 | 1,630            |    |
| D-3            | 22     | 151                       | 2,407                                                 | 590              |    |
| D-4            | 4      | 112                       | 811                                                   | 68               |    |
|                | 18,659 | 21,717                    | 50,531                                                | 171,488          |    |

It will be noted that the item prepared by diluting a double-concentration sliver at drawing had substantially more slubs per unit length and larger slubs than the item prepared with 15% slubs initially and is a closer approach to the desired slub distribution as evidenced by the commercial sample, especially in the longer lengths characteristic of antique satin.

#### EXAMPLE IV

In a manner paralleling those of the foregoing examples, two 20/2 cotton count, (~59 tex) 14 Z/7 S yarns were prepared, each comprising 90% of a commercial 2.5 denier/filament (~0.28 tex) semi-dull acrylic staple intended for spinning in the cotton system; one item (4-A) also contained 10% of 0.5 inch (~1.3-cm.) fiber nubs having the composition of component A of Example I and dried at 25° C. to have a density of about 1.14 g/cc and intense helical bicomponent crimp; the second (4-B), containing 10% of 0.5 inch (~1.3 cm) fiber nubs of the same composition dried at 155° C. to have a density of about 1.18 g/cc and only light mechanical crimp (no helical bicomponent crimp developed), is included for comparison to illustrate the poorer results obtained with fiber prepared in this prior art manner.

Uster Classimat data are:

| Class | 4-A    | 4-B |
|-------|--------|-----|
| A-1   | 8032   | 318 |
| A-2   | 462    | 24  |
| A-3   | 10     | 2   |
| A-4   | 2      | 2   |
| B-1   | 3289   | 174 |
| B-2   | 771    | 54  |
| B-3   | 26     | 9   |
| B-4   | 3      | 4   |
| C-1   | 896    | 80  |
| C-2   | 314    | 43  |
| C-3   | 24     | 15  |
| C-4   | 7      | 4   |
| D-1   | 143    | 23  |
| D-2   | 60     | 25  |
| D-3   | 13     | 20  |
| D-4   | 11     | 9   |
|       | 14,063 | 806 |

The bicomponent nubs of this invention offer substantial advantages over those currently available. An important consideration, of course, is their lower cost based on no need for special processing before incorporation into the base fiber. Special effects can also be obtained more economically because the nubs are more highly basic dyeable than ordinary acrylic fiber, and

normal basic piece-dyeing procedures will give tone-on-tone effects in acrylic yarns containing slubs derived from the nubs of this invention. Uniform or union dyeing is still within the capability of one skilled in the dyeing art, however, and this is an important aspect of the overall versatility of these nubs.

The acrylic yarns comprising slubs derived from the nubs of this invention have utility in a variety of applications. Of particular importance are curtains and drapery fabric which are outstandingly durable due to the excellent sunlight resistance of acrylic fibers generally. Others include upholstery, bedding, napery, and apparel fabrics.

We claim:

1. Process for producing a slub yarn wherein 10-50% by weight bicomponent acrylic fibers having a hydrophilic component and a less hydrophilic component and having a density of about 1.0 to 1.17 g/cm<sup>3</sup> and an equilibrium crimp reversibility of at least about 20% and cut to a length of 0.25 to 1 inch are blended with staple fibers in an amount of 50-90% by weight during or before carding and processed by conventional procedures into a slub containing spun yarn.

2. Process of claim 1 wherein the hydrophilic component is comprised of (1) 85-90% by weight acrylonitrile units, (2) 2-10% by weight units of styrene sulfonic acid (o, m or p isomer), 2-acrylamido-2-methylpropane sulfonic acid, allylsulfonic acid, methallylsulfonic acid, vinyl sulfonic acid, or their metal, ammonium or amine salts, a vinylpyridine, vinyl pyrrolidone, acrylamide, methacrylamide, hydroxymethylacrylamide or mixtures thereof (3) 0 to 13% by weight of units of a comonomer less hydrophilic than units of monomer (2).

3. Process of claim 2 wherein the less hydrophilic comonomer (3) is methyl acrylate, methyl methacrylate, vinyl acetate, methacrylonitrile or mixtures thereof.

4. Process of claim 2 wherein the less hydrophilic component of the bicomponent fibers contains 0-20% by weight of a polymer containing (1) 85-98% by weight acrylonitrile units (2) 2-10% by weight units of styrene sulfonic acid (o-, m- or p-isomer), 2-acrylamido-2-methylpropane sulfonic acid, allyl sulfonic acid, methallyl sulfonic acid, vinyl sulfonic acid or their metal, ammonium or amine salts, a vinyl pyridine, vinyl pyrrolidone, acrylamide, methacrylamide, hydroxymethylacrylamide or mixture thereof and (3) 0-13% by weight units of a comonomer less hydrophilic than units of monomer (2) and 80-100% by weight polyacrylonitrile.

5. Process of claim 4 wherein the less hydrophilic comonomer (3) is methyl acrylate, methyl methacrylate, vinyl acetate, methacrylonitrile or mixtures thereof.

6. Process of claim 1 wherein the process is carried out on the worsted system.

7. Process of claim 1 wherein the process is carried out on the cotton system.

8. Process of claim 6 wherein the bicomponent fibers are about 0.75 inches long.

9. Process of claim 7 wherein the bicomponent fibers are about 0.25 inches long.

10. Process of claim 1 wherein a card sliver containing bicomponent acrylic fibers according to claim 1 is blended with one or more card slivers which do not contain such bicomponent fibers.

11. Process of claim 1 wherein the bicomponent acrylic fibers are coated with a high friction finish.

\* \* \* \* \*